

Patented Jan. 3, 1933

## UNITED STATES PATENT OFFICE

WILLIAM ROBERT SHIMER AND FRED C. T. DANIELS, OF BETHLEHEM, PENNSYLVANIA,  
ASSIGNORS TO BETHLEHEM STEEL COMPANY

SILICO-MOLYBDENUM STEEL AND ARTICLE MADE THEREFROM

Application filed March 17, 1927. Serial No. 176,304.

No Drawing.

Our invention relates to silico-molybdenum steels, and more particularly to such steels as are applied under more or less elevated temperature conditions and where hardness together with great strength are required. Our invention consists of steels containing as the significant constituents of steels containing carbon from a low to high content, silicon, 10 .75% to 4.25% and molybdenum .15% to .75%. These steels may contain small amounts of other metals and for many purposes should contain a quantity of manganese somewhat greater than is usually present in common steels. Furthermore, some hardening agent such as chromium should be present in moderate amounts, for certain special uses.

While our invention broadly may include any proportions of the ingredients with ranges above given, for most practical purposes they should be employed within the following limits: Carbon .20% to 1.25%, silicon .80% to 2.20% and molybdenum .15% to .75%. In these steels manganese may be present between .50% to .90%, nickel up to 1.2% as the maximum and chromium up to 2.5% as the maximum. Obviously, small amounts of other elements may be added provided they do not substantially alter the essential characteristics produced by the elements specified as essential.

Our invention further consists in articles made of such compositions having great hardness and strength and certain other physical characteristics to a high degree at elevated temperatures.

We have discovered that the presence of silicon and molybdenum, within the limits above given, greatly increase the mechanical properties, such as hardness and strength. What is particularly significant is the fact that these steels possess these qualities to a remarkable degree at temperatures which are considerably elevated. Then too, these steels are considerably resistant to various disintegrating influences and tendencies at high temperatures, such as checking. Moreover, these desirable characteristics are retained

even when repeatedly subjected to widely varying and rapidly changing temperature conditions. Furthermore, these steels effectively resist great stresses, even when suddenly applied and when rapidly varying in intensity, and although these steels are hard and tough, they can be effectively machined. Several illustrative examples will now be given. For the purpose of comparing steels 60 coming within our invention with steels of known in the art, analyses are given of one of our steels together with those of silico-manganese and chromium vanadium steels as follows:

|                          | C   | Mn  | P    | S    | Si    | Cr    | Mo    | Va    |
|--------------------------|-----|-----|------|------|-------|-------|-------|-------|
| Silico-molybdenum steel. | .60 | .75 | .044 | .024 | 1.87  | .30   | .49   | ----- |
| Silico-manganese steel.  | .57 | .69 | .024 | .034 | 2.13  | ----- | ----- | ----- |
| Chromium vanadium steel. | .50 | .77 | .016 | .020 | ----- | 1.10  | ----- | .18   |

The silico-molybdenum steel was quenched in oil at 1600° F.; the silico-manganese and chromium vanadium steels were also quenched in oil at 1650° F. and 1460° F., respectively. Each of the steels were then drawn at 1000° F., the resulting product showing the following mechanical properties:

|                   | T. S.   | E. L.   | EI       | Re | Bri-nell |
|-------------------|---------|---------|----------|----|----------|
| Silico-molybdenum | 250,000 | 225,000 | Per cent | 14 | 555      |
| Silico-manganese  | 160,000 | 110,000 | 8        | 38 | 311      |
| Chromium vanadium | 159,000 | 140,000 | 18       | 55 | 375      |

When drawn at 1100° F. the materials had the following characteristics:

|                   | T. S.   | E. L.   | EI       | Red. | Bri-nell |
|-------------------|---------|---------|----------|------|----------|
| Silico-molybdenum | 235,000 | 215,000 | Per cent | 10   | 514      |
| Silico-manganese  | 148,000 | 101,000 | 20       | 43   | 262      |
| Chromium vanadium | 142,000 | 130,000 | 20       | 58   | 31       |

Drawn at 1200° F.

1,893,004

The following analyses have been found especially useful:

|                   | T. S.   | E. L.   | El       | Red.     | Bri-nell |
|-------------------|---------|---------|----------|----------|----------|
| 5                 |         |         |          |          |          |
| Silico-molybdenum | 195,000 | 180,000 | Per cent | Per cent |          |
| Silico-manganese  | 139,000 | 91,000  | 13       | 27       |          |
| Chromium vanadium | 137,000 | 117,000 | 20       | 47       | 444      |
|                   |         |         |          | 60       | 269      |
| 10                |         |         |          |          | 302      |

Drawn at 1300° F.

|                   | T. S.   | E. L.   | El       | Red.     | Bri-nell |
|-------------------|---------|---------|----------|----------|----------|
| 15                |         |         |          |          |          |
| Silico-molybdenum | 160,000 | 141,000 | Per cent | Per cent |          |
| Silico-manganese  | 130,000 | 85,000  | 17       | 37       |          |
| Chromium vanadium | 120,000 | 103,000 | 21       | 50       | 388      |
|                   |         |         | 22       | 68       | 229      |
|                   |         |         |          |          | 255      |

20 Although the prior art steels, silico manganese and chrome vanadium, above given have excellent properties, it will be seen at once that the silico-molybdenum steel of this invention has much higher physical characteristics. Note that, when drawn at 1000° F., the silico molybdenum steel has 92,000 lbs. greater tensile strength and 85,000 lbs. greater elastic limit than either of the other steels. It should be noted also that the difference in favor of our steel is maintained at the higher "draws" even at the upper figure, 1300° F. Furthermore, and this is probably the most significant fact, our steel maintains this superiority when used at elevated temperatures.

These properties make this steel almost ideal for springs, particularly for springs to be used at elevated temperatures. As is obvious, springs are frequently subjected to repeated and rapidly varying stresses. Very few materials can endure such use at high temperature. From the comparisons above given between our steel and those of other steels, which have been used for making springs, the superiority of our steels there-over is apparent, especially for purposes where the temperature is more or less elevated.

Our steels can also be very effectively used for making mill rolls, used in metal rolling. Here it is a requisite that the material of the rolls be resistant to various disintegrating influences at moderately high temperatures and that it should have great strength and hardness. While the example of our steels, which has just been given may be used for this purpose a modification thereof is more effective, as it is found that a somewhat greater carbon content and the presence of an appreciable amount of some hardening agent, such as chromium, greatly improves the usefulness of the steels for this purpose.

| C   | Mn  | P    | S    | Si   | Ni  | Cr  | Mo  |
|-----|-----|------|------|------|-----|-----|-----|
| .80 | .49 | .031 | .026 | 1.85 | .04 | .65 | .48 |
| .74 | .60 | .042 | .026 | 2.14 | .32 | .60 | .48 |

75 Rolls made of these compositions were very heat resistant, retaining their strength and hardness throughout use. They were non-checking, and when employed for sheet rolls, there was no sticking between them and the metal being rolled.

76 When chilled iron rolls are employed for rolling flat sections there are frequent breakages, but when using steels of the just given

77 These steels are also very useful for other hot work tools, such as hot punches, chisels, drop forging dies, extrusion rams, liners, etc. and the like.

78 The chromium content may be varied according to the degree of hardness desired in the finished product. Usually where considerable hardness is desired, an amount between .50% and 1% will be sufficient. Obviously, any other equivalent hardening agent may be employed providing it does not destroy the essential characteristics produced by the significant constituents of our steels, namely silicon and molybdenum.

79 The following steel has been found to be very effective in making pipe moulds, to be used for making centrifugally cast iron pipe:

| C   | Mn  | P    | S    | Si   | Ni  | Cr    | Mo  |
|-----|-----|------|------|------|-----|-------|-----|
| .29 | .86 | .039 | .021 | 2.00 | .20 | ----- | .43 |

80 Moulds made from this composition effectively resisted abrasion during the removal of the pipe from the mould. Furthermore the repeated heating and cooling of the moulds, incidental to their use, had practically no effect in causing cracking and little or no oxidation of the inside surface of the mould. Obviously these steels could be effectively used for moulds of other types.

81 In order that there be no doubt as to the construction of the claims, hereinafter written, several expressions therein used probably need more or less definition. When it is stated that silicon is present in an amount "approximately 2%" and molybde-

82 num approximately .50%" it is intended to cover any amounts substantially the same effects as the amounts actually given. For example, in the illustrations of our invention, above given, silicon is given as 1.87%, 1.85% and 2.14%. These amounts of this element produce substantially the same effects, the same effects, essentially as would be

2% of this element. Hence, the expression in the claims should not be restrictively taken. The significant thing to consider is the effect produced. What applies to the expression concerning silicon, obviously also applies to that concerning molybdenum.

By the expression "normal temperatures" it is intended to cover those of the atmosphere under ordinary circumstances.

While several examples of compositions made in accordance with our invention have been given, and also various applications thereof, obviously it is not intended to limit the invention by such illustrations. We consider that our invention broadly is the application of our discovery that silicon and molybdenum contribute high mechanical properties, such as high tensile strength and yield point, and hardness at ordinary and also at elevated temperatures. Briefly, our invention is the application of the idea that molybdenum and silicon in moderate amounts contribute great strength and hardness through a wide range of temperatures.

Having thus described our invention what we claim as new and desire to secure by Letters Patent is:

1. An article adapted to be used at both normal and elevated temperatures, and to be subjected to great stresses, made of a steel comprising carbon from .10% to 1.25%, silicon approximately 2%, molybdenum approximately .50% and chromium in substantial amounts less than 2%.

2. A mill roll made of a steel comprising silicon approximately 2%, molybdenum approximately .50% and chromium in excess of .50% but not substantially exceeding 2.00%.

3. A mill roll made of a steel comprising silicon approximately 2%, molybdenum approximately .50%, carbon greater than .65% and chromium in excess of .50% but not substantially exceeding 2.00%.

In testimony whereof I hereunto affix my

signature.

FRED C. T. DANIELS.

In testimony whereof I hereunto affix my

signature.

WILLIAM ROBERT SHIMER.